

June 18, 1974

J. B. SARDISCO

3,817,743

TREATMENT OF COPPER IRON SULFIDES TO FORM X-BORNITE

Filed Sept. 18, 1972

4 Sheets-Sheet 1



June 18, 1974

J. B. SARDISCO

3,817,743

TREATMENT OF COPPER IRON SULFIDES TO FORM X-BORNITE

Filed Sept. 18, 1972

4 Sheets-Sheet 2



June 18, 1974

J. B. SARDISCO

3,817,743

TREATMENT OF COPPER IRON SULFIDES TO FORM X-BORNITE

Filed Sept. 18, 1972

4 Sheets-Sheet 3



June 18, 1974

J. B. SARDISCO

**3,817,743**

## TREATMENT OF COPPER IRON SULFIDES TO FORM X-BORNITE

Filed Sept. 18, 1972

4 Sheets-Sheet 4



Fig. 6

1

3,817,743  
TREATMENT OF COPPER IRON SULFIDES TO  
FORM X-BORNITE  
John B. Sardisco, Shreveport, La., assignor to Pennzoil  
Company, Houston, Tex.  
Filed Sept. 18, 1972, Ser. No. 289,980  
Int. Cl. C22b 1/12, 15/08

U.S. CL. 75—1

26 Claims

## ABSTRACT OF THE DISCLOSURE

A method is described for treating chalcopyrite and other copper iron sulfides by reaction with sulfur vapor to form compositions which are more responsive to leaching. The method is amenable to continuous operation and under certain reaction conditions it may be used to produce as a principal product a granular, easy-to-handle material identified as X-bornite. Under other reaction conditions idaite is produced. The optimum reaction conditions for production of X-bornite are: (1) sulfur vapor partial pressure from about 200 mm. of Hg to about 760 mm. of Hg; (2) reaction temperature from about 460° C. to about 500° C.; and (3) residence time of at least about 6 minutes. The copper in the X-bornite and idaite can be easily solubilized with either chloride solutions or sulfuric acid solutions under oxidizing conditions. For sulfate systems copper recoveries in excess of 99% can be obtained by grinding the residue from the first leaching step to a particle size of at least about minus 200 mesh and then re-leaching.

## BACKGROUND OF THE INVENTION

### (1) Field of the Invention

This invention relates generally to hydrometallurgical processes for the production of metallic copper from copper iron sulfide ore concentrates. In particular, this invention is concerned with the treatment of copper iron sulfides to make the sulfides more responsive to hydrometallurgical processing. In accordance with this invention, chalcopyrite and other copper iron sulfides are reacted with sulfur vapor to transform these sulfides into other compounds which can be more easily leached.

### (2) Prior Art

In recent years the public and governmental agencies have become increasingly concerned with the degradation of the environment. In the western part of the United States copper smelters which process copper ore concentrates are regarded as one of the major sources of air pollution. These smelters emit gaseous streams containing particulate matter and sulfur oxides.

Sulfur oxides, which have been found very difficult to control, result from the smelting of sulfur-bearing ores. Although copper exists in various other forms in nature, such as native copper and copper oxides, carbonates and silicates, the primary sources of copper exist as low-grade deposits of copper iron sulfide ores, with the principal copper mineral being chalcopyrite.

Instead of trying to control the emissions of air contaminants, such as sulfur oxides, once they are formed, hydrometallurgical processes offer an alternative approach by avoiding the formation of the air contaminants. It has been recognized for some time that in the leaching of copper sulfide minerals, the sulfur can be recovered in solid elemental form. This is in contrast to present smelting or pyrometallurgical processes where the sulfur is removed by oxidizing the minerals at elevated temperatures, thereby forming sulfur oxides.

At the present time in the copper industry, hydrometallurgy is generally restricted to the treatment of the

2

more easily leached copper oxide ores and native copper deposits. Aside from waste-dump leaching in copper sulfide mining operations, hydrometallurgy has not been generally applied to sulfide minerals on a commercial scale. In these limited applications of hydrometallurgy, the most commonly used lixivants are sulfuric acid and ferric sulfates.

Of the copper sulfide minerals, chalcopyrite, which is the principal copper mineral in the United States, has been found to be the most resistant to treatment by hydrometallurgical processes. Processes developed for the treatment of chalcopyrite have been plagued with low recoveries of copper from the ore. Some processes have been able to recover a substantial amount of the copper in the ore but only after the leaching operation has been carried on for a number of hours which is economically undesirable. A further problem in the processing of copper iron sulfide ores is the simultaneous dissolution of the iron which acts as a contaminant in the copper recovery steps.

One attempt to make the copper iron sulfides more responsive to hydrometallurgical processes is disclosed in Vizsolyi et al., Pat. No. 3,459,535 (1969). Although the process disclosed in the Vizsolyi patent results in improved copper recovery in shorter periods of time, it does not seem amenable to commercial utilization in view of the batch operation, relatively long reaction time, material handling difficulties and failure to achieve high copper recoveries in shorter periods of time.

## SUMMARY OF THE INVENTION

The object of the present invention is to provide a means for utilizing hydrometallurgical processes for the recovery of metallic copper from copper iron sulfide ore concentrates whereby conventional pyrometallurgical processes can be replaced, thus eliminating the air pollution associated with the processing of such ore concentrates. A more particular object of the invention is the development of a process for treating copper iron sulfide ore concentrates which will make the copper iron sulfides, especially chalcopyrite, more responsive to leaching in hydrometallurgical processes. Other objects and advantages of the present invention will appear from the following description, examples and claims.

It has been discovered that these objects can be accomplished and that the difficulties of prior art processes can be obviated by treating copper iron sulfide ore concentrates with sulfur vapor, thereby forming other copper iron sulfides which can be more easily leached by conventional leaching agents, such as sulfuric acid-oxygen solutions, sulfuric acid-ferric sulfate solutions, and ferric chloride and/or cupric chloride solutions. This sulfidizing process, which takes as little as 6 minutes to complete, is preferably operated at a temperature in the range from about 460° C. to about 500° C. and at a sulfur vapor partial pressure from about 200 mm. of Hg to about 760 mm. of Hg.

In treating chalcopyrite as described, the primary product has been identified by X-ray diffraction as X-bornite. Under certain reaction conditions idaite (usually designated as  $Cu_5FeS_6$ ) has been formed. One of the discoveries of this invention has been the development of a commercial process for the production of these two relatively rare minerals.

The main advantage in reacting the ore concentrate with sulfur vapor instead of liquid sulfur is the physical form of the product. When utilizing sulfur vapor the product is in a granular or powder form, while lumps or other large pieces of product are formed when liquid sulfur is used as the starting material. The formation of a granular product which can be readily leached without further

treatment enables the sulfidizing process to be used on a continuous basis. On the other hand, the formation of relatively large pieces of product when the ore concentrate is reacted with liquid sulfur limits the practicality of the process. These large pieces tend to stick to the sides of the container and are difficult to remove. Furthermore, they must be ground to a fine particle size before they can be effectively leached within a relatively short period of time.

It has been found that by treating chalcopyrite with sulfur vapor as much as 98.5% of the copper in the chalcopyrite can be recovered by leaching with sulfuric acid-oxygen solutions in as little as two hours. If a ferric chloride and cupric chloride solution is used as the lixiviant, leaching tests have shown that as much as 98.8% of the copper goes into solution in as little as 15 minutes. Moreover, during the leaching of the reaction product from the sulfidizing process very little of the iron present as pyrite is attacked by the leaching solution, regardless whether a sulfate or a chloride solution is used.

In seeking to maximize the copper recovery, it has been found that pyrite crystals frequently prevent the copper iron sulfide from being fully exposed to the leaching solution, thus preventing solubilization of the copper in the sulfide material. To increase copper recoveries to greater than 99%, it has been discovered that grinding the residue from the initial leaching of the X-bornite or idaite to a particle size of at least about minus 200 mesh "cracks" away the pyrite crystals, thereby exposing the remaining copper iron sulfides to the leaching solution.

#### BRIEF DESCRIPTION OF THE DRAWINGS

In the accompanying drawings, FIG. 1 is a section view of a reactor that can be used in accordance with the present invention for the sulfidizing of copper iron sulfide ore concentrates.

FIG. 2 is a top view of the reaction chamber plates in the reactor of FIG. 1.

FIG. 3 is a graph showing the relationship between the reaction temperature and the chalcopyrite conversion for various partial pressures of sulfur in the sulfidizing of chalcopyrite ore concentrates.

FIG. 4 is a graph showing the optimum residence times in the sulfidizing of chalcopyrite ore concentrates.

FIG. 5 is a graph showing the percent copper extracted by sulfuric acid leaching for X-bornite and idaite as compared to non-sulfidized copper-containing materials.

FIG. 6 is a flow sheet of the process of this invention for the production of metallic copper from chalcopyrite

with sulfur vapor to form other copper iron sulfide minerals. These new products which have an increased sulfur content are substantially more responsive to leaching than chalcopyrite and other non-sulfur treated copper iron sulfide minerals.

The reactor shown in FIGS. 1 and 2 can be used to treat copper iron sulfides in accordance with the present invention. FIG. 1 is a vertical section view of a modified Herreshoff type furnace reactor 1. Heating elements 2 are used to heat the reactor and are located adjacent to the outer insulating fire brick wall 3. The ore concentrate is fed into the reactor via inlet star feeder 4 and conduit 5. Inside the stainless steel reaction chamber 6 are five stainless steel plates 7 (only the bottom plate is marked with the numeral 7 in FIG. 1), each having a slot-type opening for continuous flow of the ore concentrate. On the center shaft 8 for each plate are mounted five stainless steel scraper blades 9, as shown in FIG. 2. The ore concentrate is scraped horizontally across each plate 7 and drops vertically by gravity to the plate below, finally exiting the reaction chamber 6 as the reacted product through conduit 10 and exit star feeder 11.

Elemental sulfur which has been liquefied outside the reactor is fed through conduit 12 to sulfur flash pot 13 where it is vaporized. The vaporized sulfur is introduced into reaction chamber 6 through conduit 14. Excess sulfur vapor exits the reactor via conduits 10 and 15.

Nitrogen is introduced through conduit 16 and is used as a carrier for the sulfur vapor and in controlling the partial pressure of sulfur vapor. Additional nitrogen is introduced into conduits 5 and 10 at 17 and 18, respectively, to maintain a nitrogen atmosphere in the reaction chamber 6 and to aid in controlling the sulfur partial pressure.

The principal copper containing product (at least about 70% by weight) has been concluded to be X-bornite based upon the description of X-bornite found in an article by Yund and Kullerud entitled "Thermal Stability of Assemblages in the Cu-Fe-S System," Journal of Petrology, Vol. 7, Part 3, pp. 454-88 (1966). Pyrite as well as some bornite  $Cu_5FeS_4$  and idaite  $Cu_5FeS_6$  are also formed. The two principal products, pyrite and X-bornite, generally comprise at least about 85% by weight of the reaction product. Table I below presents X-ray diffraction pattern data for material produced by sulfidizing chalcopyrite ore concentrate in accordance with this invention as compared to the data presented for X-bornite in the Yund et al. article and standard data for bornite, pyrite and other minerals.

TABLE I

| Pattern data of sample |     |       |           | Standard data for— |          |         |                  |         |              |   |          |
|------------------------|-----|-------|-----------|--------------------|----------|---------|------------------|---------|--------------|---|----------|
| $^{\circ}2\theta$      | I   | D     | X-bornite | Pyrite             | Idaite   | Bornite | $SiO_2$ (quartz) | $MoS_2$ | Chalcopyrite |   |          |
|                        | D   | D     | I/I max.  | D                  | I/I max. | D       | I/I max.         | D       | I/I max.     | D | I/I max. |
| 14.58                  | 30  | 6.11  |           |                    |          |         |                  | 6.15    | 100          |   |          |
| 20.92                  | 15  | 4.24  |           |                    |          |         | 4.26             | 35      |              |   |          |
| 26.68                  | 60  | 3.34  |           |                    |          |         | 3.343            | 100     |              |   |          |
| 27.60                  | 50  | 3.23  |           |                    |          |         |                  |         |              |   |          |
| 27.98                  | 40  | 3.19  |           |                    |          |         |                  |         |              |   |          |
| 28.56                  | 150 | 3.12  | 3.11      | 48                 | 3.128    | 36      | 3.134            | 100     |              |   |          |
| 29.40                  | 45  | 3.04  |           |                    |          |         |                  |         |              |   |          |
| 31.84                  | 20  | 2.808 |           |                    |          |         | 2.818            | 80      |              |   |          |
| 32.80                  | 25  | 2.728 |           |                    |          |         |                  | 2.74    | 50           |   |          |
| 33.10                  | 260 | 2.704 | 2.699     | 43                 | 2.709    | 84      |                  |         |              |   |          |
| 37.12                  | 150 | 2.420 |           |                    |          |         | 2.423            | 66      |              |   |          |
| 40.80                  | 110 | 2.210 |           |                    |          |         | 2.212            | 52      |              |   |          |
| 47.00                  | 30  | 1.932 |           |                    |          |         |                  | 1.937   | 100          |   |          |
| 47.50                  | 210 | 1.912 | 1.910     | 100                | 1.916    | 40      |                  |         |              |   |          |
| 48.20                  | 30  | 1.886 |           |                    |          |         |                  | 1.887   | 65           |   |          |
| 56.32                  | 150 | 1.632 | 1.630     | 21                 | 1.633    | 100     |                  |         |              |   |          |
| 59.10                  | 15  | 1.562 | 1.559     | 7                  | 1.564    | 14      |                  |         |              |   |          |
| 61.72                  | 30  | 1.502 |           |                    |          |         | 1.502            | 20      |              |   |          |
| 64.30                  | 30  | 1.447 |           |                    |          |         | 1.448            | 24      |              |   |          |

NOTE:  $2\theta$ =angle of detection. I=Intensity in counts per second. D=interplanar spacing in Angstrom units. I/I max.=relative intensity in percent. ore concentrates utilizing sulfuric acid as the leaching agent.

#### DESCRIPTION OF THE PREFERRED EMBODIMENTS

In accordance with the present invention chalcopyrite and other copper iron sulfide ore concentrates are reacted

70 The material for which X-ray diffraction data are presented in Table I was produced by treating chalcopyrite ore concentrate with sulfur vapor maintained at a partial pressure of 200 mm. of Hg for 13 minutes. The reaction temperature was 471° C. and sulfur/copper molar ratio of the feed material to the reactor was 1.3. The chalco-

pyrite ore concentrate used in this example as well as in the other examples reported herein was obtained from Duval Corporation's Sierrita mine near Tucson, Ariz. A wet chemical analysis of this ore concentrate showed 1.13% acid soluble copper, 2.48% non-chalcopyrite copper, 23.23% chalcopyrite copper, 28.1% iron and 30.3% sulfur.

With reference to the X-ray diffraction data presented in Table I, it can be seen that some of the X-bornite peaks overlap some of the pyrite peaks which prevents a positive identification of the material as either pyrite or X-bornite. For example, the peak at a  $2\theta$  value of 47.50° has a much higher intensity relative to the peak at the  $2\theta$  value of 56.32° than it has in a known pyrite sample. The peak at the  $2\theta$  value of 47.50° in the Table I sample is about 140% of the peak at the  $2\theta$  value of 56.32°, while in a known pyrite sample it is only about 40% of the peak at the  $2\theta$  value of 56.32°.

Consequently, to obtain a more positive identification of the X-bornite, a known sample of bornite was reacted with sulfur vapor under similar reaction conditions. The only different reaction condition was the use of a 1.0 sulfur/copper molar feed ratio. The X-ray diffraction data for the product material is presented in Table II and indicates, based on the data from the Yund et al article, that the material is X-bornite.

TABLE II

| Pattern data of sample |           |       | Standard data for—      |          |       |          |   |          |
|------------------------|-----------|-------|-------------------------|----------|-------|----------|---|----------|
| $^{\circ}2\theta$      | X-bornite |       | $\text{SiO}_2$ (quartz) |          |       |          | D | I/I max. |
|                        | I         | D     | D                       | I/I max. | D     | I/I max. |   |          |
| 20.98                  | 40        | 4.23  | 4.23                    | —        | 4.26  | 35       |   |          |
| 26.76                  | 170       | 3.33  | 3.33                    | —        | 3.343 | 100      |   |          |
| 28.66                  | 200       | 3.11  | 3.11                    | 48       | —     |          |   |          |
| 33.16                  | 180       | 2.699 | 2.699                   | 43       | —     |          |   |          |
| 47.58                  | 420       | 1.910 | 1.910                   | 100      | —     |          |   |          |
| 56.38                  | 90        | 1.680 | 1.680                   | 21       | —     |          |   |          |
| 59.20                  | 30        | 1.559 | 1.559                   | 7        | —     |          |   |          |

The true relationship of X-bornite to bornite is not

TABLE III

| Pattern data of sample |         |       | Standard data for— |          |           |          |       |          |                         |                  |              |          |
|------------------------|---------|-------|--------------------|----------|-----------|----------|-------|----------|-------------------------|------------------|--------------|----------|
| $^{\circ}2\theta$      | Bornite |       | Pyrite             |          | X-bornite |          | D     | I/I max. | $\text{SiO}_2$ (quartz) | MoS <sub>2</sub> | Chalcopyrite |          |
|                        | I       | D     | D                  | I/I max. | D         | I/I max. | D     | I/I max. | D                       | I/I max.         | D            | I/I max. |
| 14.50                  | 10      | 6.10  | —                  |          | —         |          | —     |          | —                       | —                | 6.15         | 100      |
| 20.98                  | 15      | 4.23  | 4.23               | —        | —         |          | 4.26  | 35       | —                       | —                | —            |          |
| 21.84                  | 10      | 4.07  | 4.08               | 10       | —         |          | —     |          | —                       | —                | —            |          |
| 26.72                  | 60      | 3.33  | 3.33               | —        | —         |          | 3.343 | 100      | —                       | —                | —            |          |
| 27.04                  | 20      | 3.29  | 3.31               | 40       | —         |          | —     |          | —                       | —                | —            |          |
| 27.56                  | 50      | 3.23  | 3.23               | —        | —         |          | —     |          | —                       | —                | —            |          |
| 27.98                  | 50      | 3.19  | 3.18               | 60       | —         |          | —     |          | —                       | —                | —            |          |
| 28.32                  | 50      | 3.15  | 3.15               | —        | —         |          | —     |          | —                       | —                | —            |          |
| 28.58                  | 100     | 3.12  | 3.128              | —        | 36        | 3.11     | 48    | 3.134    | 100                     | —                | —            |          |
| 29.46                  | 25      | 3.03  | 3.03               | —        | —         |          | —     |          | —                       | —                | 3.03         | 100      |
| 31.68                  | 20      | 2.822 | 2.822              | —        | —         |          | 2.818 | 80       | —                       | —                | —            |          |
| 31.98                  | 15      | 2.796 | 2.80               | 20       | —         |          | 2.792 | 60       | —                       | —                | —            |          |
| 32.80                  | 50      | 2.728 | 2.74               | 50       | —         |          | —     |          | —                       | —                | —            |          |
| 33.06                  | 195     | 2.707 | 2.707              | —        | 2.709     | 84       | 2.699 | 43       | —                       | —                | —            |          |
| 35.74                  | 20      | 2.610 | 2.50               | 40       | —         |          | —     |          | —                       | —                | —            |          |
| 37.12                  | 100     | 2.420 | 2.423              | 66       | —         |          | —     |          | —                       | —                | —            |          |
| 40.84                  | 90      | 2.208 | 2.212              | 52       | —         |          | —     |          | —                       | —                | —            |          |
| 47.00                  | 90      | 1.932 | 1.937              | 100      | —         |          | —     |          | —                       | —                | —            |          |
| 47.50                  | 140     | 1.912 | 1.916              | 40       | 1.910     | —        | 100   | —        | —                       | —                | —            |          |
| 55.74                  | 20      | 1.648 | 1.652              | 30       | —         |          | —     |          | —                       | —                | —            |          |
| 56.34                  | 200     | 1.632 | —                  | —        | 1.633     | 100      | 1.630 | 21       | —                       | —                | —            |          |
| 59.06                  | 25      | 1.563 | —                  | —        | 1.564     | 14       | 1.559 | 7        | —                       | —                | —            |          |
| 61.70                  | 35      | 1.502 | —                  | —        | 1.502     | 20       | —     | —        | —                       | —                | —            |          |
| 64.32                  | 35      | 1.447 | —                  | —        | 1.448     | 24       | —     | —        | —                       | —                | —            |          |

NOTE:  $2\theta$ =angle of detection. I=intensity in counts per second. D=interplanar spacing in Angstrom units. I/I max.=relative intensity in percent. exactly clear, as is indicated in the Yund article. Yund and Kullerud suggest that X-bornite contains slightly more sulfur than stoichiometric bornite  $\text{Cu}_5\text{FeS}_4$ . The reaction of sulfur with chalcopyrite to produce X-bornite is probably similar to the reaction producing bornite which is as follows:



During theoretical phase relation studies, Yund and Kullerud were able to produce X-bornite by annealing sulfur-rich synthetic bornites at a temperature below approximately 140° C. Although X-bornite occurs in some geological environments, there is no suggestion in the

Yund article or other prior art of the means for producing X-bornite on a commercial basis as is disclosed herein.

The reaction temperature for producing X-bornite can range from the temperature at which sulfur vaporizes, about 440° C., to about 530° C. The optimum temperature for sulfidizing chalcopyrite ore concentrates has been found to be in the range from about 460° C. to about 500° C.

In treating chalcopyrite ore concentrates, partial pressures of sulfur above approximately 200 mm. of Hg promote the reaction with chalcopyrite. Increasing the sulfur partial pressure from about 200 mm. of Hg to about one atmosphere does not seem to affect the reaction one way or the other. Sufficient sulfur should be initially fed to the reaction vessel to maintain the partial pressure at approximately 200 to 760 mm. of Hg. It has been found that this can usually be accomplished by using a sulfur/copper molar feed ratio from about 1.2 to about 1.6. To keep the desired sulfur partial pressure additional sulfur is supplied during the reaction to provide for replacement of the reacted sulfur. FIG. 3 shows the percent conversion of chalcopyrite as a function of temperature and sulfur partial pressure.

A minimum residence time (defined as the time the ore remains in the reactor) of about 6 minutes is necessary for obtaining a high conversion of chalcopyrite during the sulfidizing reaction at optimum conditions. This is shown by FIG. 4. This graph in FIG. 4 also indicates that an increase in the residence time has no significant effect in reducing the amount of residual chalcopyrite in the reaction product.

If the reaction product consisting primarily of X-bornite is kept at the reaction temperature under a nitrogen atmosphere for an additional period of time, a different product is formed which is primarily bornite. This can be seen from Table III which shows X-ray diffraction data for the final reaction product resulting from heating sulfidized chalcopyrite at 471° C. for 12 minutes in a nitrogen atmosphere.

TABLE III

| Standard data for— |         |       |        |          |           |          |       |          |                         |                  |              |     |
|--------------------|---------|-------|--------|----------|-----------|----------|-------|----------|-------------------------|------------------|--------------|-----|
| $^{\circ}2\theta$  | Bornite |       | Pyrite |          | X-bornite |          | D     | I/I max. | $\text{SiO}_2$ (quartz) | MoS <sub>2</sub> | Chalcopyrite |     |
|                    | I       | D     | D      | I/I max. | D         | I/I max. |       |          |                         |                  |              |     |
| 14.50              | 10      | 6.10  | —      |          | —         |          | —     |          | —                       | —                | 6.15         | 100 |
| 20.98              | 15      | 4.23  | 4.23   | —        | —         |          | 4.26  | 35       | —                       | —                | —            |     |
| 21.84              | 10      | 4.07  | 4.08   | 10       | —         |          | —     |          | —                       | —                | —            |     |
| 26.72              | 60      | 3.33  | 3.33   | —        | —         |          | 3.343 | 100      | —                       | —                | —            |     |
| 27.04              | 20      | 3.29  | 3.31   | 40       | —         |          | —     |          | —                       | —                | —            |     |
| 27.56              | 50      | 3.23  | 3.23   | —        | —         |          | —     |          | —                       | —                | —            |     |
| 27.98              | 50      | 3.19  | 3.18   | 60       | —         |          | —     |          | —                       | —                | —            |     |
| 28.32              | 50      | 3.15  | 3.15   | —        | —         |          | —     |          | —                       | —                | —            |     |
| 28.58              | 100     | 3.12  | 3.128  | —        | 36        | 3.11     | 48    | 3.134    | 100                     | —                | —            |     |
| 29.46              | 25      | 3.03  | 3.03   | —        | —         |          | —     |          | —                       | —                | 3.03         | 100 |
| 31.68              | 20      | 2.822 | 2.822  | —        | —         |          | 2.818 | 80       | —                       | —                | —            |     |
| 31.98              | 15      | 2.796 | 2.80   | 20       | —         |          | 2.792 | 60       | —                       | —                | —            |     |
| 32.80              | 50      | 2.728 | 2.74   | 50       | —         |          | —     |          | —                       | —                | —            |     |
| 33.06              | 195     | 2.707 | 2.707  | —        | 2.709     | 84       | 2.699 | 43       | —                       | —                | —            |     |
| 35.74              | 20      | 2.610 | 2.50   | 40       | —         |          | —     |          | —                       | —                | —            |     |
| 37.12              | 100     | 2.420 | 2.423  | 66       | —         |          | —     |          | —                       | —                | —            |     |
| 40.84              | 90      | 2.208 | 2.212  | 52       | —         |          | —     |          | —                       | —                | —            |     |
| 47.00              | 90      | 1.932 | 1.937  | 100      | —         |          | —     |          | —                       | —                | —            |     |
| 47.50              | 140     | 1.912 | 1.916  | 40       | 1.910     | —        | 100   | —        | —                       | —                | —            |     |
| 55.74              | 20      | 1.648 | 1.652  | 30       | —         |          | —     |          | —                       | —                | —            |     |
| 56.34              | 200     | 1.632 | —      | —        | 1.633     | 100      | 1.630 | 21       | —                       | —                | —            |     |
| 59.06              | 25      | 1.563 | —      | —        | 1.564     | 14       | 1.559 | 7        | —                       | —                | —            |     |
| 61.70              | 35      | 1.502 | —      | —        | 1.502     | 20       | —     | —        | —                       | —                | —            |     |
| 64.32              | 35      | 1.447 | —      | —        | 1.448     | 24       | —     | —        | —                       | —                | —            |     |

Under optimum reaction conditions the amount of residual chalcopyrite in the reaction product is approximately 1-3% by wet chemical analysis. To further reduce the residual chalcopyrite, the reaction product can be recycled through the reactor and treated as described above. However, the main product of such recycling is idaite instead of X-bornite. As will be discussed later, idaite is similar to X-bornite in its responsiveness to leaching. Table IV presents X-ray diffraction data for the reaction product of recycling the initial reaction product at 471° C. for 13 minutes. The sulfur/copper molar feed

ratio was 1.39 and the sulfur partial pressure was maintained at 208 mm. of Hg.

Solid sulfur and chalcopyrite ore concentrate were inserted into the reactor and then heated to 475° C. The resulting

TABLE IV

| Standard data for—     |     |        |       |          |        |          |     |           |     |          |                           |          |              |          |                  |          |
|------------------------|-----|--------|-------|----------|--------|----------|-----|-----------|-----|----------|---------------------------|----------|--------------|----------|------------------|----------|
| Pattern data of sample |     | Idaite |       |          | Pyrite |          |     | X-bornite |     |          | SiO <sub>2</sub> (quartz) |          | Chalcopyrite |          | MoS <sub>2</sub> |          |
| ° 2θ                   | I   | D      | D     | I/I max. | D      | I/I max. | D   | I/I max.  | D   | I/I max. | D                         | I/I max. | D            | I/I max. | D                | I/I max. |
| 14.52                  | 35  | 6.10   |       |          |        |          |     |           |     |          |                           |          |              |          | 6.15             | 1001     |
| 20.00                  | 15  | 4.44   |       |          |        |          |     |           |     |          |                           |          |              |          |                  |          |
| 20.96                  | 15  | 4.23   |       |          |        |          |     |           |     |          |                           |          |              |          |                  |          |
| 23.90                  | 20  | 3.72   | 3.723 | 10       |        |          |     |           |     |          | 426                       | 35       |              |          |                  |          |
| 26.68                  | 35  | 3.34   |       |          |        |          |     |           |     |          |                           |          |              |          |                  |          |
| 27.32                  | 55  | 3.26   | 3.265 | 25       |        |          |     |           |     |          | 3.343                     | 100      |              |          |                  |          |
| 27.62                  | 40  | 3.23   |       |          |        |          |     |           |     |          |                           |          |              |          |                  |          |
| 28.06                  | 55  | 3.18   |       |          |        |          |     |           |     |          |                           |          |              |          |                  |          |
| 28.54                  | 230 | 3.12   | 3.134 | 100      | 3.128  |          | 36  | 3.11      | 48  |          |                           |          |              |          |                  |          |
| 29.46                  | 20  | 3.03   |       |          |        |          |     |           |     |          |                           |          |              |          |                  |          |
| 31.74                  | 160 | 2.817  | 2.818 | 80       |        |          |     |           |     |          |                           |          |              |          |                  |          |
| 32.04                  | 130 | 2.791  | 2.792 | 60       |        |          |     |           |     |          |                           |          |              |          |                  |          |
| 33.14                  | 220 | 2.701  |       |          | 2.709  |          | 84  | 2.699     | 43  |          |                           |          |              |          |                  |          |
| 36.60                  | 20  | 2.453  | 2.456 | 6        |        |          |     |           |     |          |                           |          |              |          |                  |          |
| 37.16                  | 125 | 2.417  |       |          | 2.423  |          | 66  |           |     |          |                           |          |              |          |                  |          |
| 40.86                  | 125 | 2.207  |       |          | 2.212  |          | 52  |           |     |          |                           |          |              |          |                  |          |
| 42.52                  | 20  | 2.124  | 2.123 | 8        |        |          |     |           |     |          |                           |          |              |          |                  |          |
| 47.52                  | 130 | 1.912  |       |          | 1.916  |          | 40  | 1.910     | 100 |          |                           |          |              |          |                  |          |
| 48.20                  | 155 | 1.886  | 1.887 | 65       |        |          |     |           |     |          |                           |          |              |          |                  |          |
| 49.36                  | 115 | 1.845  | 1.845 | 65       |        |          |     |           |     |          |                           |          |              |          |                  |          |
| 56.34                  | 205 | 1.632  |       |          | 1.633  |          | 100 | 1.630     | 21  |          |                           |          |              |          |                  |          |
| 56.92                  | 35  | 1.616  | 1.618 | 10       |        |          |     |           |     |          |                           |          |              |          |                  |          |
| 59.04                  | 80  | 1.563  | 1.564 | 30       | 1.564  |          | 14  | 1.559     | 7   |          |                           |          |              |          |                  |          |
| 61.74                  | 45  | 1.501  |       |          | 1.502  |          | 20  |           |     |          |                           |          |              |          |                  |          |
| 64.36                  | 55  | 1.446  |       |          | 1.448  |          | 24  |           |     |          |                           |          |              |          |                  |          |

NOTE: 2θ=angle of detection. I=intensity in counts per second. D=interplanar spacing in Angstrom units. I/I max.=relative intensity in percent.

The sulfidizing of chalcopyrite and other copper iron sulfide minerals is especially adaptable to continuous processing techniques. The reaction time is relatively short and the reaction product can be easily handled and transported since it is in granular form.

In contrast to the vapor-phase reaction of the present invention, the liquid-phase reaction of the prior art, that is, heating a mixture of solid sulfur and copper iron sulfide ore concentrates to the point where the sulfur is liquefied and even possibly vaporized, results in a reaction product which presents difficult material handling problems. Large pieces of product, which has been found to be mainly idaite, are formed, and frequently the product sticks to and fouls the walls of the reaction vessels. Consequently, before leaching the liquid-phase reaction product must be ground to a fine particle size. In addition, due to the fouling of the reaction vessel the liquid-phase reaction presents difficulties for normal batch and continuous processing.

In the vapor-phase sulfidizing of chalcopyrite, the particle size of the products is actually less than that of the incoming chalcopyrite ore concentrate. For example, the mass mean diameter of the chalcopyrite ore concentrate particles was 0.091 mm. with only 48 weight percent passing through a 200 mesh screen. After vapor-phase sulfidizing the chalcopyrite ore concentrate, the mass mean diameter of the resulting product particles was 0.068 mm. with 87 weight percent passing through a 200 mesh screen.

The objective of the sulfidizing reaction is to produce a copper iron sulfide material from which the copper can be quickly leached in appreciable quantities by conventional leaching agents, such as sulfuric acid-oxygen solutions, sulfuric acid-ferric sulfate solutions, and ferric chloride and/or cupric chloride solutions, at relatively low pressures and temperatures.

A method for pressure leaching of chalcopyrite with sulfuric acid and oxygen is reported by Vizsolyi et al. at page 52 of the November 1967 issue of the Journal of Metals. To obtain at least 98 percent solubilization of the chalcopyrite within three hours, the particles had to be ground to a size where 99.5% passed through 325 mesh screen and 50% stoichiometric excess of sulfuric acid was required. The oxygen partial pressure and temperature were maintained at 500 p.s.i. and 116° C., respectively.

In U.S. pat. No. 3,459,535, Vizsolyi et al. described a process for leaching a covellite-pyrite material with oxygen and sulfuric acid at 90° C. and 70 p.s.i. of oxygen. The covellite-pyrite material was prepared by reacting sulfur with chalcopyrite in a batch reactor at 475° C. for 2 hours.

45 material had to be broken up and ground before leaching to a particle size of substantially 100% minus 325 mesh. During the leaching step, five hours of residence time was required to obtain copper extractions greater than 98.5 weight percent, and under these conditions 53 weight percent of the iron from the pyrite was leached.

By my invention over 98.5% of the copper can be solubilized in as little as two hours by leaching the sulfidized copper iron sulfides with sulfuric acid and oxygen. 50 For one set of examples, the copper iron sulfides from the vapor phase reactor were not ground as in prior art processes but were only screened to remove the plus 100 mesh size particles and then pressure leached in an autoclave using only one stage. Table V below shows: (A) the 55 composition of the copper iron sulfides resulting from the vapor phase sulfidizing of chalcopyrite ore concentrates; (B) results of leaching tests on sulfidized ore; (C) results of leaching tests on chalcopyrite ore; and (D) reaction conditions for these leaching tests.

60 TABLE V.—CONDITIONS AND RESULTS FOR PRESSURE LEACHING USING SULFURIC ACID AND OXYGEN  
A.—Compositions of the copper iron sulfides (sulfidized ore)

| Sulfidized ore sample | West chemical analyses (wt. percent) |       |       | X-ray diffraction analysis                                       |    |   |
|-----------------------|--------------------------------------|-------|-------|------------------------------------------------------------------|----|---|
|                       | Cu                                   | Fe    | S     | Cu                                                               | Fe | S |
| No. 1.....            | 24.71                                | 24.19 | 36.19 | 2-3% chalcopyrite; remainder is X-bornite and pyrite.            |    |   |
| No. 2.....            | 24.71                                | 24.90 | 36.10 | 4-5% chalcopyrite; 3% idaite; remainder is X-bornite and pyrite. |    |   |

70 B.—Leaching tests on sulfidized ore

| Test No. | Sulfidized ore sample No. | Residence time (hrs.) | Wt. percent solubilized |      |     | Material balance (wt. percent) |      |      |
|----------|---------------------------|-----------------------|-------------------------|------|-----|--------------------------------|------|------|
|          |                           |                       | Cu                      | Fe   | S   | Cu                             | Fe   | S    |
| 1.....   | 1                         | 2                     | 98.5                    | 27.0 | 0.2 | 104.8                          | 90.8 | 97.6 |
| 2.....   | 1                         | 2.5                   | 98.8                    | 27.0 | 1.3 | 103.9                          | 92.1 | 99.3 |
| 3.....   | 2                         | 2                     | 99.0                    | 37.1 | 8.0 | 95.0                           | 86.5 | 97.1 |

75 C.—Leaching tests on chalcopyrite ore

| Test No. | Residence time (hrs.) | Wt. percent solubilized |      |       | Material balance (wt. percent) |       |       |
|----------|-----------------------|-------------------------|------|-------|--------------------------------|-------|-------|
|          |                       | Cu                      | Fe   | S     | Cu                             | Fe    | S     |
| 4.....   | 2                     | 57.1                    | 24.1 | -17.4 | 127.5                          | 104.8 | 107.0 |
| 5.....   | 2                     | 55.4                    | 31.3 | -10.4 | 112.1                          | 98.8  | 100.7 |

35 NOTE: For Test No. 4, the chalcopyrite was dried at 475° C. in a nitrogen atmosphere prior to leaching.

D.—Reaction conditions

Temperature: 70° C.

Oxygen partial pressure: 90 p.s.i.

Stirrer speed: 1,500 r.p.m.

Wt. percent of sulfuric acid in leach liquor: 13.0%.

Grams of leach liquor per gram of sulfidized ore: 3.76.

It can be seen from Table V that only 55-57% copper is solubilized when leaching chalcopyrite ore as compared to 98.5-99.0% solubilization when leaching sulfidized ore. Moreover, only 27-37% of the iron in the sulfidized ore was solubilized.

The data in Table VI show the advantage of leaching X-bornite or idaite over native bornite or covellite ore. All the leaching tests were made at an oxygen partial pressure of 70 p.s.i. and 105° C. using about 13.0 wt. percent sulfuric acid and 3.7 grams of acidic solution per gram of ore material. Stirrer speed was 1500 r.p.m. and particle size of the ore material was minus 200 plus 325 mesh. Table VI and FIG. 5 show the results of these leaching tests and illustrate the significant difference in the leaching characteristics of the different materials. The sulfidized materials, idaite and X-bornite, are considerably more susceptible to acid leaching than the other materials.

TABLE VI.—CONDITIONS AND RESULTS FOR PRESSURE LEACHING USING SULFURIC ACID AND OXYGEN

| Test number | Material leached       | Residence time (hrs.) | Initial wt. percent H <sub>2</sub> SO <sub>4</sub> | Material balance (wt. percent) |       |       | Chemical analysis of spent residue |      |       |     |                     |                      |                        |
|-------------|------------------------|-----------------------|----------------------------------------------------|--------------------------------|-------|-------|------------------------------------|------|-------|-----|---------------------|----------------------|------------------------|
|             |                        |                       |                                                    | Cu                             | Fe    | Su    | Wt. percent solubilized            | Cu   | Fe    | S   | Acid soluble copper | Copper as chalcocite | Copper as chalcopyrite |
| 1           | X-bornite <sup>1</sup> | 1                     | 12.98                                              | 101.7                          | 96.6  | 93.3  | 97.0                               | 30.6 | 11.6  | .51 | .43                 | .3                   |                        |
| 2           | do <sup>1</sup>        | 1.5                   | 12.98                                              | 102.8                          | 101.1 | 95.1  | 95.1                               | 27.5 | 10.2  | .45 | .39                 | .25                  |                        |
| 3           | do <sup>1</sup>        | 2                     | 12.98                                              | 102.3                          | 99.4  | 97.7  | 98.5                               | 37.4 | 11.7  | .34 | .14                 | .15                  |                        |
| 4           | Native covellite       | 1                     | 12.98                                              | 94.1                           | 87.7  | 96.4  | 58.0                               | 19.6 | .84   |     |                     |                      |                        |
| 5           | do <sup>1</sup>        | 1.5                   | 13.13                                              | 93.1                           | 83.8  | 94.2  | 67.0                               | 24.9 | -4.7  |     |                     |                      |                        |
| 6           | do <sup>1</sup>        | 2                     | 13.13                                              | 92.5                           | 85.2  | 91.3  | 79.2                               | 26.8 | -5.1  |     |                     |                      |                        |
| 7           | Native bornite         | 1                     | 13.13                                              | 100.1                          | 118.9 | 97.4  | 79.2                               | 38.7 | -44.1 |     |                     |                      |                        |
| 8           | do <sup>1</sup>        | 1.5                   | 13.13                                              | 102.3                          | 103.0 | 90.6  | 87.0                               | 72.0 | -39.5 |     |                     |                      |                        |
| 9           | do <sup>1</sup>        | 2                     | 13.13                                              | 99.8                           | 100.4 | 94.2  | 92.6                               | 78.1 | -33.7 |     |                     |                      |                        |
| 10          | Idaite <sup>2</sup>    | 1.5                   | 12.97                                              | 101.3                          | 103.4 | 102.2 | 93.8                               | 20.9 | 3.2   |     |                     |                      |                        |
| 11          | do <sup>2</sup>        | 2                     | 12.97                                              | 97.0                           | 103.4 | 105.1 | 94.3                               | 21.0 | -3.7  |     |                     |                      |                        |
| 12          | do <sup>2</sup>        | 2                     | 13.13                                              | 101.0                          | 104.0 | 98.7  | 95.9                               | 24.1 | 5.8   | .39 | 1.09                | .21                  |                        |
| 13          | do <sup>2</sup>        | 1.5                   | 13.13                                              | 105.3                          | 104.2 | 87.1  | 89.8                               | 18.2 | 13.1  | .23 | 3.52                | .34                  |                        |
| 14          | do <sup>2</sup>        | 2.5                   | 13.13                                              | 102.2                          | 98.6  | 95.0  | 97.0                               | 33.5 | 11.1  | .34 | .73                 | .21                  |                        |

<sup>1</sup> Composition by X-ray diffraction is mainly X-bornite and pyrite with about 4% chalcopyrite and some idaite.

<sup>2</sup> Composition by X-ray diffraction is mainly idaite and pyrite with about 1% chalcopyrite and some X-bornite and bornite (vapor-phase preparation).

TABLE VII.—CONDITIONS AND RESULTS FOR THE TWO-STAGE LEACHING TESTS

| Test No. | Material leached     | Stage | Size of material | Total pressure p.s.i. | Residence time hr. | Gms. H <sub>2</sub> SO <sub>4</sub> per gms. Cu | Wt. percent solubilized across one stage |      |      | Wt. percent solubilized across both stages |       |       | Material balance across one stage (wt. percent) |      |   |
|----------|----------------------|-------|------------------|-----------------------|--------------------|-------------------------------------------------|------------------------------------------|------|------|--------------------------------------------|-------|-------|-------------------------------------------------|------|---|
|          |                      |       |                  |                       |                    |                                                 | Cu                                       | Fe   | S    | Cu                                         | Fe    | S     | Cu                                              | Fe   | S |
| 1        | 1 X-bornite          | —100  | 88               | 2                     | 2.0                | 96.6                                            | 48.2                                     | 23.6 |      | 103.4                                      | 92.7  | 93.2  |                                                 |      |   |
|          | 2 Residue stage 1... | —325  | 88               | 1                     | 59.5               | 92.0                                            | 39.9                                     | 24.5 | 99.7 | 68.8                                       | 42.3  | 81.5  | 86.9                                            | 89.9 |   |
| 2        | 1 X-bornite          | —100  | 88               | 3                     | 2.0                | 82.7                                            | 48.7                                     | 24.8 |      | 110.4                                      | 92.8  | 91.8  |                                                 |      |   |
|          | 2 Residue stage 1... | —325  | 88               | 2                     | 11.8               | 94.7                                            | 47.1                                     | 29.0 | 99.1 | 72.9                                       | 46.6  | 107.3 | 98.5                                            | 81.2 |   |
| 3        | 1 X-bornite          | —100  | 88               | 3                     | 2.0                | 96.1                                            | 55.3                                     | 29.4 |      | 105.1                                      | 90.8  | 90.6  |                                                 |      |   |
|          | 2 Residue stage 1... | —325  | 88               | 1                     | 29.7               | 87.2                                            | 34.5                                     | 17.5 | 99.5 | 70.7                                       | 41.7  | 92.4  | 97.7                                            | 88.1 |   |
| 4        | 1 X-bornite          | —100  | 68               | 2                     | 2.0                | 93.7                                            | 44.5                                     | 24.6 |      | 97.0                                       | 82.6  | 88.6  |                                                 |      |   |
|          | 2 Residue stage 1... | —325  | 68               | 2                     | 32.3               | 91.5                                            | 44.8                                     | 30.8 | 99.5 | 69.4                                       | 47.9  | 90.7  | 98.0                                            | 88.8 |   |
| 5        | 1 X-bornite          | —190  | 68               | 1                     | 2.0                | 87.2                                            | 28.8                                     | 5.9  |      | 114.0                                      | 87.9  | 92.9  |                                                 |      |   |
|          | 2 Residue stage 1... | —200  | 68               | 1                     | 15.9               | 67.6                                            | 23.4                                     | 16.3 | 95.8 | 46.2                                       | 21.3  | 98.0  | 103.9                                           | 89.8 |   |
| 6        | 1 X-bornite          | —100  | 88               | 1                     | 2.0                | 89.5                                            | 35.4                                     | 8.9  |      | 112.5                                      | 87.7  | 92.7  |                                                 |      |   |
|          | 2 Residue stage 1... | —200  | 88               | 1                     | 19.3               | 75.7                                            | 27.9                                     | 15.4 | 97.4 | 53.9                                       | 23.0  | 101.6 | 101.0                                           | 91.0 |   |
| 7        | 1 X-bornite          | —100  | 88               | 2                     | 2.0                | 95.8                                            | 49.8                                     | 22.1 |      | 106.6                                      | 88.8  | 91.0  |                                                 |      |   |
|          | 2 Residue stage 1... | —200  | 88               | 1                     | 49.2               | 78.2                                            | 29.2                                     | 15.3 | 99.1 | 64.4                                       | 34.0  | 101.7 | 102.6                                           | 95.9 |   |
| 8        | 1 X-bornite          | —325  | 88               | 2                     | 2.0                | 95.7                                            | 37.7                                     | 15.0 |      | 102.8                                      | 108.5 | 93.9  |                                                 |      |   |
|          | 2 Residue stage 1... | —325  | 68               | 2                     | 47.7               | 94.0                                            | 55.7                                     | 26.7 | 99.7 | 72.4                                       | 37.6  | 85.4  | 89.4                                            | 88.0 |   |

In attempting to maximize the copper recovery, it was found through the use of microphotographs that pyrite crystals are imbedded at random in the crystals of the sulfidized copper iron sulfides during the vapor-phase reaction. In some cases 2-3% of the total copper is entrapped, in the form of copper iron sulfide crystals, by the pyrite crystals and is thus shielded from the leaching solution. Accordingly, another object of this invention is to provide a method for leaching the copper entrapped by the pyrite crystals.

I have unexpectedly discovered that by grinding the residue from a one-stage pressure leach reaction, during which most (at least about 80%) of the copper was solubilized, the pyrite crystals can be "cracked" away, thereby exposing the remaining copper iron sulfides to the leaching agents. By this method I can solubilize sub-

60 65

The resulting pregnant liquor from the pressure leach reaction contains an appreciable amount of iron which must be removed before the copper sulfate solution can be treated by electrolysis to produce metallic copper. Excess iron in the electrolytic cell reduces the cathode efficiency and can contribute to contamination of the copper.

It has been found that the iron can be removed by precipitating it as a jarositic iron oxide-sulfate. The ratio of sulfate ions to iron in the combined precipitate has been found to be essentially that of the compound jarosite. It is precipitated from an acid solution at pH values of 1.5 and above. Since the pregnant liquor from the leach reaction contains excess sulfuric acid, the pH values range from 0.5 to 1.0. Thus, before jarosite can be precipitated the excess sulfuric acid must be neutralized. In the present invention the neutralization of the sulfuric acid can be ac-

complished with cement or scrap copper according to the following equation:



The oxidation state of iron in jarosite is +3, thus any ferrous ions in the liquor must be oxidized to ferric ions. This is accomplished by oxidation with oxygen as follows:



Sodium ions for the jarosite formation can be supplied by such sodium compounds as sodium hydroxide or sodium carbonate. When sodium hydroxide is used, it is believed that the reaction proceeds as below:



The reactions above can be carried out in one reactor, or the cement copper and the sodium hydroxide can be added prior to the oxidation step. The reaction has been carried out in a standard autoclave in which the pressure leach tests were conducted. The pregnant liquor, cement copper, and sodium hydroxide were placed in the autoclave at the same time. The temperature was increased and oxygen was then applied under pressure.

High temperature was used because it produced a more easily filterable precipitate. The oxidation rate of the ferrous ions to ferric ions increased with the use of high pressure.

A number of runs were made during which about 80 percent of the iron in the pregnant liquor was removed. Very little copper remained in the residue with the iron. For these tests, enough cement copper was added to the liquor to bring the pH up to 1.5-2.0, and enough sodium hydroxide was added to satisfy the reaction of equation (4). The conditions for carrying out these tests were as follows:

Temperature: 115° C.

Contact Time: 2 hrs.

Partial Pressure of Oxygen: 70 p.s.i.

Total Pressure: 95 p.s.i.

Stirrer Speed: 1,500 r.p.m.

Table VIII below contains the conditions and results of these tests.

TABLE VIII.—CONDITIONS AND RESULTS FOR IRON REMOVAL TESTS

| Test No. | Gms. of liquid feed | Liquid feed (wt. percent) |      |       | Gms. of cement | Gms. of copper | 100% NaOH | Liquid product (wt. percent) |       |       | Spent residue (wt. percent) | Material balance (wt. percent) |       |       |
|----------|---------------------|---------------------------|------|-------|----------------|----------------|-----------|------------------------------|-------|-------|-----------------------------|--------------------------------|-------|-------|
|          |                     | Cu                        | Fe   | S     |                |                |           | Cu                           | Fe    | S     |                             | Cu                             | Fe    | S     |
| 1        | 300                 | 5.65                      | 1.40 | 4.29  | 9.0            | 0.3            | 4.43      | .14                          | 1.89  | 1.5   | 1.4                         | 45.2                           | 120.8 | 113.8 |
| 2        | 300                 | 6.20                      | 1.04 | 3.60  | 2.0            | 2.0            | 3.86      | .11                          | 1.69  | 1.45  | 1.6                         | 39.6                           | 121.1 | 105.8 |
| 3        | 300                 | 5.89                      | 1.89 | 4.27  | 3.0            | 1.1            | 5.89      | .16                          | 3.2   | 1.1   | 0.9                         | 28.1                           | 98.3  | 85.1  |
| 4        | 600                 | 5.75                      | 1.96 | ----- | 9.0            | 2.0            | 6.32      | .29                          | ----- | 1.1   | 1.0                         | 30.9                           | 102.7 | 94.3  |
| 5        | 600                 | 5.65                      | 1.72 | 4.04  | 10.75          | 2.2            | 7.29      | .29                          | 3.72  | ----- | 1.2                         | 26.3                           | 9.23  | 90.8  |
| 6        | 600                 | 5.65                      | 1.12 | 3.51  | 10.0           | 1.0            | 4.47      | .16                          | ----- | 1.5   | 2.6                         | 25.3                           | ----- | 101.9 |
| 7        | 1,263               | 9.03                      | 1.79 | 5.87  | 30             | 4.8            | 4.39      | .14                          | 2.08  | ----- | 1.3                         | 17.1                           | 4.4   | 81.8  |
| 8        | 300                 | 6.94                      | 1.85 | 5.58  | 0              | 15             | 6.37      | .24                          | 4.89  | ----- | 3.4                         | 29.3                           | 12.9  | 98.8  |

NOTE.—Analysis of cement copper used in wt. percent: Cu—83.6%, Fe—8.0%, S—0.4%.

After about 80% of the iron has been removed from the pregnant liquor, the solution contains approximately 6-8% copper, 0.2-0.4% iron, and 1-3% free sulfuric acid. The copper in this solution can be recovered in metallic form by conventional electrowinning methods. Equation (5) sets forth the reaction in the electrolytic cell:



About 60% of the copper in the copper sulfate solution is removed during electrolysis at the following conditions:

Temperature: 30-50° C.

Contact Time: 14-21 hrs.

Voltage: 1.6-2.5 volts

Current Density: 7 to 25 (amps/sq. ft.)

Current Efficiency: About 85%

The conditions and results of typical electrowinning tests are shown in Table IX:

TABLE IX.—RESULTS AND CONDITIONS FOR ELECTROWINNING TESTS

| Test number                         | 1    | 2    | 3   |
|-------------------------------------|------|------|-----|
| Conditions:                         |      |      |     |
| Temperature (° C.)                  | 30   | 30   | 30  |
| Voltage (volts)                     | 2.0  | 2.0  | 2.3 |
| Current density (amps/sq. ft.)      | 7.0  | 7.0  | 25  |
| Liquid feed (wt. percent):          |      |      |     |
| Cu                                  | 3.5  | 3.5  | 3.4 |
| Fe                                  | 0.13 | 0.4  | 0.6 |
| S                                   | 4.3  | 4.3  | 4.5 |
| Contact time (hrs.)                 | 21   | 21   | 9   |
| Results:                            |      |      |     |
| Current efficiency (percent)        | 88   | 71   | 78  |
| Percent copper removed              | 61   | 51   | 54  |
| Rate of copper depletion (gms./hr.) | 1.2  | 0.97 | 2.3 |

Another advantage of the above-described method is that the purification of cement or scrap copper can be incorporated into the overall process. As was discussed previously, cement or scrap copper is added to the system to neutralize excess sulfuric acid in the iron removal step.

One embodiment of the process according to the present invention wherein sulfuric acid is used as the leaching agent is shown by the flow diagram in FIG. 6.

In treating chalcopyrite ore concentrates, the ore concentrates are added to sulfidizing reactor 101 through line 102. Molten sulfur is introduced into reactor 101 through line 103 wherein it is vaporized before being mixed with the ore concentrates. The vaporized sulfur is preferably maintained at a partial pressure of at least about 200 mm. of Hg. In the reactor the ore concentrates are sulfidized in as little as six minutes at a temperature of about 470° C., thereby converting most of the chalcopyrite to X-bornite and pyrite. Excess sulfur is discharged through line 104.

The sulfidized ore from reactor 101 is then passed through line 105 to primary leach stage 106, into which is also passed sulfuric acid solution through line 107 and oxygen sufficient to maintain a partial pressure of about 90 p.s.i. through line 108. The acid oxidation leach solution at a temperature of about 105° C. solubilizes most of the copper in the ore in about two hours.

The leach slurry from the primary leach stage is then transported through line 109 to primary separation device

110. In this device the solids consisting primarily of a small amount of unreacted copper iron sulfides, elemental sulfur and insoluble residue are separated from the solution containing copper sulfate, ferrous sulfate and unreacted sulfuric acid. The solids are transported through line 111 to grinding stage 112 and the solution goes to iron removal stage 114 through line 113.

In the grinding stage the solids are further ground by use of conventional size reduction equipment to at least about minus 200 mesh. The ground solids are then transported to secondary leach stage 116 through line 115.

To solubilize essentially all the remaining copper in the copper iron sulfides, oxygen is added to the secondary leach stage through line 117 and regenerated sulfuric acid solution is added through line 118. The reaction conditions are essentially the same as those in the primary leach stage. The resulting slurry is then transported to secondary separation device 120 through line 119.

In device 120 conventional separation means are used to separate the solution containing excess sulfuric acid, ferrous sulfate and copper sulfate from the solid material consisting primarily of elemental sulfur and insoluble residue which is discharged through line 121. If desired the elemental sulfur can be separated from the residue by means known to those skilled in the art. The solution is discharged from device 120 through line 122 and is combined with the regenerated sulfuric acid solution that is added to the primary leach stage through line 107.

In iron removal stage 114 the pregnant liquor containing copper sulfate, ferrous sulfate and excess sulfuric acid is first treated to neutralize the excess sulfuric acid by the addition of cement copper through line 123. Oxygen sufficient to maintain a partial pressure of about 70 p.s.i. is added through line 124 to oxidize the ferrous ions to ferric ions and sodium hydroxide is added through line 125 to precipitate the ferric iron as jarositic iron oxide-sulfate. The preferred reaction temperature is 115° C. and the normal contact time is about 1-2 hours.

The slurry from iron removal stage 114 is transported through line 126 to iron separation device 127 wherein the jarositic material is separated from the solution containing primarily copper sulfate and some ferric sulfate. The jarositic material is discharged through line 128 and the solution is transported through line 129 to electrolytic cells 130. The jarositic material may alternatively be recycled to either the primary or the secondary leach stage for the removal of any copper therein. In such case the jarositic precipitate would be removed from the process with the insoluble residue.

The solution in cells 130 is electrolyzed to produce metallic copper and to regenerate sulfuric acid. Metallic copper is removed at 131 and the regenerated sulfuric acid solution which is used in both the secondary and primary leach stages is discharged through line 107.

The X-bornite and idaite prepared by the process according to the present invention offers a considerable advantage in the use of ferric chloride and/or cupric chloride as the leaching agent. Considerably more copper can be leached from X-bornite or idaite than chalcopyrite during a given period of time. Table X contains conditions and results for atmospheric pressure leaching of X-bornite and chalcopyrite using ferric chloride and cupric chloride, along with sodium chloride which acts to keep cuprous chloride in solution and is believed to aid the reaction.

TABLE X.—CONDITIONS AND RESULTS FOR ATMOSPHERIC PRESSURE LEACHING USING FERRIC CHLORIDE AND CUPRIC CHLORIDE

A.—Reaction conditions

Temperature: About 110° C.

Pressure: Atmospheric.

Grams FeCl<sub>3</sub>/grams sulfidized ore: 1.

Grams CuCl<sub>2</sub>·2H<sub>2</sub>O/grams sulfidized ore: 0.2.

Grams H<sub>2</sub>O/grams sulfidized ore: 2.8.

Sulfidized ore composition: By wet chemical analysis—26.23% Cu, 25.14% Fe and 38.00% S. By X-ray diffraction analysis, 4% chalcopyrite, about 2% bornite, about 4% idaite, with the remainder being X-bornite and pyrite.

B.—Leaching tests on sulfidized ore

| Test No. | Gms.<br>ore | Gms.<br>NaCl/<br>gms.<br>ore | Reaction<br>time<br>(hrs.) | Wt. percent<br>solubilized | Material<br>balance (wt.<br>percent) |       |
|----------|-------------|------------------------------|----------------------------|----------------------------|--------------------------------------|-------|
|          |             |                              |                            |                            | Cu                                   | Fe    |
| 1.       | 0.8         | 0.5                          | 98.7                       | 14.5                       | 105.6                                | 102.7 |
| 2.       | 0.8         | 0.25                         | 98.8                       | 17.2                       | 101.8                                | 95.5  |
| 3.       | 1.0         | 0.25                         | 99.4                       | 26.2                       | 89.4                                 | 92.4  |

C.—Leaching tests on chalcopyrite ore

| Test No. | Gms.<br>ore | Gms.<br>NaCl/<br>gms.<br>ore | Reaction<br>time<br>(hrs.) | Wt. percent<br>solubilized | Material<br>balance (wt.<br>percent) |      |
|----------|-------------|------------------------------|----------------------------|----------------------------|--------------------------------------|------|
|          |             |                              |                            |                            | Cu                                   | Fe   |
| 4.       | 1.0         | 0.25                         | 51.3                       | 44.2                       | 108.5                                | 93.8 |
| 5.       | 0.8         | 0.25                         | 51.6                       | 46.5                       | 108.8                                | 99.4 |

NOTE.—The residue cake was washed by re-slurrying with dilute hydrochloric acid.

Note from Table X the fast rate of the dissolution reaction with X-bornite. Within 15 minutes more than 98.5% of the copper was solubilized. Under the same conditions only 51% of the copper in the chalcopyrite was leached.

5 What is claimed is:

1. In the processing of copper iron sulfide ore concentrates for the hydrometallurgical production of metallic copper wherein the ore concentrates are leached with a chloride solution, an improved method of making the copper iron sulfides in the ore concentrates more responsive to said chloride leaching solution which comprises reacting sulfur vapor with the ore concentrates to form a reaction product with at least about 70% of the copper-containing material in the reaction product being X-bornite.

10 2. The method according to claim 1 wherein the sulfur vapor has a partial pressure of at least about 200 mm. of Hg and the reaction temperature is in the range from about 460° C. to about 500° C.

15 3. The method according to claim 2 wherein the ore concentrates consist primarily of chalcopyrite ore concentrates and the chloride leaching solution contains ferric chloride and cupric chloride.

20 4. In the processing of chalcopyrite ore concentrates for the hydrometallurgical production of metallic copper wherein chalcopyrite ore concentrates are leached with a sulfate solution, an improved method of making the chalcopyrite in the ore concentrates more responsive to said sulfate leaching solution which comprises reacting sulfur vapor with the ore concentrates at a sulfur partial pressure of at least about 200 mm. of Hg and at a reaction temperature in the range from about 440° C. to about 530° C. for such a period of time as to form a reaction product with at least about 70% of the copper-containing material in the reaction product being X-bornite.

25 5. The method according to claim 4 wherein the sulfate leaching solution contains sulfuric acid and oxygen.

6. The method according to claim 5 wherein the reaction temperature is in the range from about 460° C. to about 500° C.

30 7. In the processing of copper iron sulfide ore concentrates for the hydrometallurgical production of metallic copper, the method of solubilizing substantially all of the copper in the copper iron sulfides which comprises:

35 (a) reacting sulfur vapor with the ore concentrates to form a reaction product consisting principally of copper-containing material and pyrite, with at least about 70% of the copper-containing material being X-bornite;

40 (b) leaching the reaction product from step (a) to solubilize most of the copper in the reaction product;

(c) grinding the solid residue from step (b) to a particle size of at least about minus 200 mesh; and

45 (d) leaching the ground residue from step (c) to solubilize substantially all the remaining copper in the reaction product.

50 8. The method according to claim 7 wherein the leaching in both steps (b) and (d) is performed with a sulfuric acid solution under oxidizing conditions.

60 9. The method according to claim 8 wherein the ore concentrates consist primarily of chalcopyrite ore concentrates.

65 10. The method according to claim 9 wherein the sulfur vapor is maintained in step (a) at a partial pressure of at least about 200 mm. of Hg and the reaction temperature for step (a) is in the range from about 440° C. to about 530° C.

70 11. The method according to claim 7 wherein the leaching is performed with a ferric chloride-cupric chloride solution.

12. A method for the hydrometallurgical production of metallic copper from copper iron sulfide ore concentrates which comprises:

(a) reacting sulfur vapor with the ore concentrates to form a reaction product with at least about 70%

of the copper-containing material in the reaction product with at least about 70% of the copper-containing material in the reaction product being X-bornite;

- (b) leaching the reaction product from step (a) with a sulfuric acid solution under oxidizing conditions to solubilize most of the copper in the reaction product;
- (c) grinding the solid residue from step (b) to a particle size of at least about minus 200 mesh;
- (d) leaching the ground residue from step (c) with a sulfuric acid solution under oxidizing conditions to solubilize substantially all the remaining copper in the reaction product of step (a);
- (e) oxidizing the solution containing the solubilized copper to precipitate iron from the solution; and
- (f) electrolyzing the solution from which the iron has been precipitated to produce metallic copper and to regenerate sulfuric acid solution for reuse in the leaching steps.

13. The method according to claim 12 wherein the solution containing the solubilized copper is reacted with cement copper to raise the pH of the solution to at least 1.5 and wherein oxygen and a material selected from the group consisting of sodium carbonate and sodium hydroxide are added to the solution to precipitate the iron in the form of jarositic iron oxide-sulfate.

14. The method according to claim 13 wherein the oxidation step (step (e)) is performed at a temperature of at least about 115° C. and at an oxygen partial pressure of about 70 p.s.i.

15. The method of claim 12 wherein the ore concentrates consist primarily of chalcopyrite ore concentrates.

16. The method of claim 15 wherein the sulfur vapor reacted with the ore concentrates in step (a) is maintained at a partial pressure of at least about 200 mm. of Hg and the reaction temperature for step (a) is in the range from about 460° C. to about 500° C.

17. The method of claim 16 wherein only the solution containing the solubilized copper from step (b) is oxidized in step (e) and the solution containing the solubilized copper from step (d) is recycled along with the regenerated sulfuric acid solution from step (f) to step (b).

18. A method for the hydrometallurgical production of metallic copper from copper iron sulfide ore concentrates containing primarily chalcopyrite which comprises:

- (a) reacting the ore concentrates with sulfur vapor at a partial pressure of at least about 200 mm. of Hg and at a temperature in the range from about 460° C. to about 500° C. for at least about 6 minutes to form a granular reaction product with at least about 70% of the copper-containing material in the reaction product being X-bornite;
- (b) leaching the reaction product from step (a) with a sulfuric acid solution under oxidizing conditions to form a slurry containing sulfur, solids, excess sulfuric acid, copper sulfate, and ferrous sulfate, thereby solubilizing most of the copper in the reaction product of step (a);
- (c) separating the sulfur and the solids in the slurry of step (b) from the solution containing the copper sulfate, ferrous sulfate and excess sulfuric acid;
- (d) grinding the solids and sulfur from step (c) to a particle size of at least about minus 200 mesh;
- (e) leaching the ground solids and sulfur from step (d) with a sulfuric acid solution under oxidizing conditions to form a slurry containing sulfur, solids, copper sulfate, ferrous sulfate, and excess sulfuric acid, thereby solubilizing substantially all the remaining copper in the reaction product of step (a);
- (f) separating the sulfur and solids in the slurry of step (e) from the solution containing the copper sulfate, ferrous sulfate and excess sulfuric acid;

(g) reacting cement copper with the solution of step (c) to raise the pH of the solution to at least about 1.5;

- (h) reacting sodium hydroxide and oxygen at a partial pressure of at least about 70 p.s.i. with the solution of step (g) at a temperature of at least about 115° C. to precipitate iron in the form of jarositic iron oxide-sulfate;
- (i) electrolyzing the solution from which the iron has been precipitated to produce metallic copper and to regenerate sulfuric acid solution; and
- (j) recycling the sulfuric acid solution of step (i) to step (e) and along with the solution of step (f) to step (b) for use in further leaching.

19. In a hydrometallurgical process for treating copper iron sulfide ore concentrates for the production of metallic copper comprising sulfidizing the ore concentrates, leaching the sulfidized ore concentrates to solubilize the copper and recovering metallic copper from the leach solution, the improvement wherein said sulfidizing comprises reacting sulfur vapor with the ore concentrates to form a reaction product with at least about 70% of the copper-containing material in the reaction product being X-bornite.

20. The method according to claim 19 wherein the ore concentrates consist essentially of chalcopyrite ore concentrates and the reaction product comprises principally copper-containing material and pyrite.

21. The method according to claim 19 wherein the ore concentrates consist essentially of bornite ore concentrates.

22. The method according to claim 19 wherein the X-bornite is further reacted with additional sulfur vapor to form idaite.

23. The method according to claim 19 wherein the sulfur vapor is maintained at a partial pressure in the range from about 200 mm. of Hg to about 760 mm. of Hg.

24. The method according to claim 23 wherein the reaction temperature is in the range from about 440° C. to about 530° C.

25. The method according to claim 24 wherein the reaction is maintained for at least about 6 minutes.

26. In a hydrometallurgical process for treating copper iron sulfide ore concentrates containing primarily chalcopyrite ore concentrates for the production of metallic copper comprising sulfidizing the ore concentrates, leaching the sulfidized ore concentrates to solubilize the copper and recovering metallic copper from the leach solution, the improvement wherein said sulfidizing comprises reacting the ore concentrates with sulfur vapor at a partial pressure of above about 200 mm. of Hg and at a temperature in the range from about 460° C. to about 500° C. for at least about 6 minutes to form a reaction product with at least about 70% of the copper-containing material in the reaction product being X-bornite.

#### References Cited

##### UNITED STATES PATENTS

|           |         |                 |          |
|-----------|---------|-----------------|----------|
| 3,637,371 | 1/1972  | Mackin et al.   | 75—117 X |
| 2,746,859 | 5/1956  | McGauley et al. | 75—1 X   |
| 3,351,462 | 11/1967 | Arentzen et al. | 75—73 X  |
| 3,169,853 | 2/1965  | Van Es          | 75—104 X |
| 1,736,659 | 11/1929 | Mitchell        | 75—104 X |
| 3,574,599 | 4/1971  | Orloff et al.   | 75—104   |
| 3,490,899 | 1/1970  | Krivosky        | 75—72 X  |
| 3,656,937 | 4/1972  | Gandon et al.   | 75—117 X |

##### FOREIGN PATENTS

|           |        |               |       |
|-----------|--------|---------------|-------|
| 1,059,476 | 2/1967 | Great Britain | 75—2  |
| 3,191     | 1905   | Great Britain | 75—74 |

ALLEN B. CURTIS, Primary Examiner

U.S. CL. X.R.

UNITED STATES PATENT OFFICE  
CERTIFICATE OF CORRECTION

Patent No. 3,817,743 Dated June 18, 1974

Inventor(s) John B. Sardisco

It is certified that error appears in the above-identified patent and that said Letters Patent are hereby corrected as shown below:

Col. 3, Table I, first numeral under 20 Column heading, "14.58" should read -- 14.48 --

Col. 7, Table IV, first numeral under MoS<sub>2</sub>, I/I max. column heading, "1001" should read -- 100 --

Col. 7, line 86, "pat." should be -- Pat. --

Col. 8, Table V., the heading "West chemical analyses" should be -- Wet chemical analyses --

Col. 9, Table VI., first numeral under Copper as chalcopyrite column heading, ".3" should be -- .30 --

Col. 9, Table VI., under Material balance (wt. percent) column, "Su" should be -- S --

Col. 9, Table VI., Test 2, under Wt. percent solubilized, Cu column, "95.1" should be -- 97.5 --

Col. 9, Table VII., under the column heading Wt. percent solubilized across one stage, above the third column of numerals (after "Fe"), add -- S -- as a column heading.

Col. 9, Table VII., Test 2, "state" should be -- stage --.

Col. 9, Table VII., Test 5, under Size of material column, "190" should be -- -100 --

Col. 9, line 63, "vapor-phase reaction" should be -- vapor-phase sulfidizing reaction --

Col. 13, line 12, "sulfrate" should be -- sulfate --

UNITED STATES PATENT OFFICE  
CERTIFICATE OF CORRECTION

Patent No. 3,817,743 Dated June 18, 1974

Inventor(s) John B. Sardisco

It is certified that error appears in the above-identified patent and that said Letters Patent are hereby corrected as shown below:

Col. 15, lines 2-3, the phrase "with at least about 70% of the copper-containing material in the reaction product" is repeated.

Col. 16, line 5, "prsssure" should be -- pressure --.

Signed and sealed this 14th day of January 1975.

(SEAL)

Attest:

McCOY M. GIBSON JR.  
Attesting Officer

C. MARSHALL DANN  
Commissioner of Patents